

## UNITED STATES PATENT OFFICE

1,925,557

PHOTOGRAPHIC DEVELOPER WITH  
ALKALI SUBSTITUTEMerle L. Dundon, Rochester, N. Y., assignor to  
Eastman Kodak Company, Rochester, N. Y.,  
a corporation of New YorkNo Drawing. Application February 2, 1932  
Serial No. 590,520

6 Claims. (Cl. 95—88)

This invention relates to a photographic developer and particularly to one in which the usual alkalies are substituted by a class of compounds new for the purpose.

- 5 Alkaline developers have now been known and used for many years. These developers usually contain developing agents, a so-called preservative, such as sodium sulphite, and alkalies, such as sodium or potassium carbonates, or sodium or potassium hydroxides. In recent years various sensitive materials and photographic processes have appeared with which the use of these stronger alkalies is objectionable for one reason or another. It is an object of this invention to provide 10 substances which may be used in a photographic developer in place of these stronger alkalies and to provide developers giving satisfactory results without the objectionable features of those containing the alkalies previously used.
- 15 Substances which I have found suitable as alkali substitutes are the alkyl amines, particularly those containing one or more hydroxy alkyl groups. Triethanolamine and its homologues are 20 representative examples. Of this preferred class of substances the following are especially useful:

## 1. Monoethanolamine



## 2. Diethanolamine



## 3. Triethanolamine

4.  $\beta$ -diethylamino ethyl alcohol

45 Of these, triethanolamine is commercially available and is very satisfactory. It may be used in certain types of developers in which borax is used as the alkali or in other combinations where it replaces the stronger alkalies mentioned.

50 Another substance included within the scope of my invention is the following:

## 5. Tri-n-propylamine



55 The following formulas will serve to illustrate my invention:

## Example I

|                                   |           |
|-----------------------------------|-----------|
| Monomethylparaminophenol sulphate | 2 grams   |
| Hydroquinone                      | 5 grams   |
| Sodium sulphite                   | 100 grams |
| Triethanolamine, 90% solution     | 2 c. c.   |
| Water to                          | 1 liter   |

## Example II

|                                   |            |
|-----------------------------------|------------|
| Monomethylparaminophenol sulphate | 0.75 grams |
| Hydroquinone                      | 3.75 grams |
| Sodium sulphite                   | 30.0 grams |
| Triethanolamine, 90% solution     | 15 c. c.   |
| Water to                          | 1 liter    |

In formulas such as these, triethanolamine acts not only as an alkali, but prevents excessive sludging in the developer.

Some of the substances included in my broad definition are not useful because they are not sufficiently soluble in the developer. Thus, the homologues of triethanolamine above propanolamine are not sufficiently soluble to be useful. The tertiary amines,



in which each R is an alkyl group, are soluble when each alkyl group does not contain more than 3 carbon atoms. The soluble compounds, 90 however, function very satisfactorily.

I consider as included in my invention all modifications and equivalents coming within the scope of the appended claims.

## What I claim is:

1. A photographic developer comprising a developing agent and a compound having the general formula



where any R may be an alkyl group, or an hydroxy alkyl group, and X is a hydroxy alkyl group.

2. A photographic developer comprising a developing agent and an alkyl amine containing one or more hydroxy alkyl groups.

3. A photographic developer comprising in solution a developing agent and as the only alkali an alkyl amine containing one or more hydroxy alkyl groups.

4. A photographic developer comprising a developing agent and triethanolamine.

5. A photographic developer comprising a developing agent and triethanolamine as the only alkali.

6. A photographic developer comprising a developing agent, a preservative, and triethanolamine.

MERLE L. DUNDON. 120